

Patented Sept. 22, 1925.

## UNITED STATES PATENT OFFICE.

CURT PHILIPP AND RICHARD FEIBELMANN, OF RADEBEUL, AND ROBERT HALLER, OF GROSSENHAIN, GERMANY, ASSIGNORS TO CHEMISCHE FABRIK VON HEYDEN, OF RADEBEUL-DRESDEN, GERMANY, A CORPORATION OF GERMANY.

## PROCESS FOR BLEACHING VEGETABLE, ANIMAL, AND ARTIFICIAL FIBERS.

No Drawing.

Application filed January 3, 1925. Serial No. 422.

To all whom it may concern:

Be it known that we, CURT PHILIPP and RICHARD FEIBELMANN, both citizens of the Republic of Germany, residing at Radebeul, 5 Saxony, and ROBERT HALLER, a citizen of the Republic of Switzerland, residing at Grossenhain, Saxony, Germany, have invented certain new and useful Improvements in Processes for Bleaching Vegetable, Animal, 10 and Artificial Fibers, of which the following is a specification.

This invention relates to bleaching processes and it particularly relates to processes in which a number of materials of greatly 15 varying character, for instance vegetable fibers such as cotton, flax, straw, hemp, raffia, jute, sisal and the like fibers in their raw state or in the form of intermediate or finished goods made from them, dyed or 20 printed textile goods are treated with the salts of the aromatic sulfochloramides, preferably in the form of their aqueous solution. Also animal fibers, such as wool in the raw state or in the form of intermediate or finished goods made from it, furs, feathers, 25 leather, horn, ivory and the like, as well as artificial fibers, like artificial silk and the many artificial substitutes for ivory, if reduced to thin threads, or thin sheets, may be 30 bleached by means of the salts of the aromatic sulfochloramides. We have found that the aforesaid salts may be applied with excellent results as a bleaching agent, the effect of these agents being mild which allows 35 several very important advantages. For instance cotton and linen fibers are not affected by our process, if treated at a high temperature; even the fiber of artificial silk, known to be very sensitive to moisture and 40 chemical agents, is not reduced in strength; it may even be applied for bleaching under pressure which is of great importance in the bowking and debasting as our invention makes it possible to have the bowking and 45 debasting process accompanied by a bleaching process.

The bleaching effect of the salts of the sulfochloramides is based on the gradual generation of oxygen according to the following 50 equation:



in which  $\text{Me}^{\text{I}}$  represents a mono-valent metal, 55

for instance such as sodium, and R represents an aromatic nucleus, such as benzene, toluene and the like. 60

It is a special merit of our process that metal oxides, which in other bleaching processes are often dangerous to the fiber on account of the catalytic action caused by the same, are without any action whatever in 65 our new process.

For the better understanding of our invention we are going to describe by way of example, how we proceed to carry the same into effect. 70

## Example 1.—Bleaching of washing.

100 kilo soiled washing is acted upon for half an hour in a bath, with 30—50 g. of the sodium-salt of p-toluenesulfochloramide 75



at a temperature of 50—100° C., the presence of soap and sodium-carbonate in the bath accelerating the cleaning process. The aforesaid p-tolue-sulfochloramide-sodium 80 dissolves the dirt, but it acts especially as a bleaching agent in such manner that the lawn-bleach may be entirely dispensed with. Old washing with a yellow tinge turns white again. 85

Our invention shortens the washing process whereby the material of the washing is not exposed to the mechanical treatment for such a long time as heretofore.

After the washing has been boiled, it is 90 rinsed and dried. The washing thus treated is distinguished by a fresh pleasant scent.

## Example 2.—Bleaching textile fabrics.

The raw goods, printed with indigo on a white ground, are worked in a bath of 95 slightly acid reaction, containing in 1000 liters of water 1 Ko. of p-tolue-sulfochloramide-sodium. The printed color gets richer and the white ground shows up brighter so as to considerably enhance the 100 appearance of the goods.

It is possible to combine the bleaching process with that of applying the mordant.

## Example 3.

The goods dyed with indigo are printed 105 simultaneously with an organic acid and a catalyst, for which purpose compound of copper, iron, cobalt, nickel, vanadium and

of other metals were found suitable. For instance we reduce 100 g. of a neutral thickening agent such as starch, 50 g. lactic acid and 10 g. copper sulfide (CuS) to a paste and 5 use the same as printing dye. With this paste the dyed goods are printed. After 10 drying the material is passed through a hot mordanting bath containing 10% p-toluene-sulfochloramide sodium. The mordanting 15 takes place very quickly.

*Example 4.*

The fabric, dyed with Columbia-black, a direct cotton dye, is treated with a printing 20 paste containing for each 100 g. thickening agent 50 gr. tartaric acid and 10 gr. iron-chloride. The mordanting is carried out as 25 in example 3.

*Example 5.—Bleaching of artificial silk.*

The raw artificial silk, which in the same 20 factory is not always obtained, batch for batch, in the same shade, is given an equalizing bleach by passing the threads at any 25 convenient temperature through a bath of approximately 0.1—0.5% p-toluene-sulfochloramide-sodium, the amount of the same being governed by the desired grade of 30 bleaching. The strength of the thread is not reduced.

Also the bleaching of straw, flax, cellulose, leather and other vegetable and animal 30 materials can be accomplished in a similar manner. In some cases, as for instance of leather, it is advantageous to add some acid to the bleaching liquid.

*Example 6.—Bleaching of cotton under pressure. (bowking process).*

Vegetable fiber or fabric is heated in a 40 boiler with an alkaline liquid of for instance 2.5° Bé. containing for each liter of the bath 1 g. p-toluene-sulfochloramide-sodium. This so-called bowking process causes a considerable preliminary bleaching effect without the formation of oxycellulose and allows a reduction of the time of the bowking 45 process.

*Example 7.*

Degumming and bleaching is done simultaneously by saturating the goods in a hot 50 bath containing approximately 0.1—0.5% p-toluene-sulfochloramide-sodium and allowing them to stand in wooden tanks, the latter kind of tanks being preferable so as to preserve a temperature of about 70—80° C. for one hour.

*Example 8.—Cleaning and bleaching of raw wool.*

Raw wool is washed with an aqueous solu-

tion of 0.5 percent of sodium carbonate and of 0.5 percent of p-toluenesulfochloramide at a temperature of 40—50° C. It is then 60 taken from the bath, washed with water and dried. In this manner the wool is well cleaned from fatty products and at the same time bleached.

What we claim is:

1. The process of treating vegetable, animal and artificial fibers, said process comprising acting on the fibers with the salt of an aromatic sulfohalogenamide.

2. The process of treating vegetable, animal and artificial fibers, said process comprising acting on the fibers with the aqueous solution of a salt of an aromatic sulfohalogenamide.

3. The process of treating vegetable, animal and artificial fibers, said process comprising acting on the fibers at an elevated temperature with a solution of a salt of an aromatic sulfohalogenamide.

4. The process of treating vegetable, animal and artificial fibers, said process comprising acting on the fibers at an elevated temperature with a solution of a salt of an aromatic sulfohalogenamide under pressure.

5. The process of treating fibers, comprising the step of acting on the fibers with a solution of a salt of an aromatic sulfohalogenamide in the presence of an acid.

6. The process of treating vegetable, animal and artificial fibers, said process comprising acting on the fibers with the solution of the sodium salt of p-toluenesulfochloramide.

7. The process of treating vegetable, animal and artificial fibers, said process comprising acting on the fibers at an elevated temperature with the solution of the sodium salt of p-toluenesulfochloramide.

8. The process of treating vegetable, animal and artificial fibers, said process comprising acting on the fibers at an elevated temperature with the solution of the sodium salt of p-toluenesulfochloramide under pressure.

9. The process of treating fibers, comprising the step of acting on the fibers with the solution of the sodium salt of p-toluenesulfochloramide in the presence of an acid.

In testimony whereof we affix our signatures.

CURT PHILIPP.  
RICHARD FEIBELMANN.  
ROBERT HALLER.